

## UNITED STATES PATENT OFFICE

1,952,090

## CASE-HARDENING METALS

Ernest C. Moffett, Woodbridge, N. J., assignor to  
American Cyanamid Company, New York, N. Y.,  
a corporation of Maine

No Drawing. Application July 11, 1931,  
Serial No. 550,287

8 Claims. (Cl. 148—15)

This invention relates to case-hardening of metals and is more particularly directed to a composition forming a molten bath in which metals are immersed for the purpose of hardening the surface thereof.

Sodium cyanide has frequently been used, either alone, or mixed with sodium chloride and sodium carbonate for case-hardening steel. The depth of case, the hardness, etc. obtainable by the use of such mixtures are well-known. However, it is further known that efficient case-hardening does not take place with such materials unless a relatively high concentration of sodium cyanide is used and maintained. Thus, the usual case-hardening bath for steel contains at least 25% of sodium cyanide and preferably higher percentages. The molten bath of the usual type containing sodium cyanide has many other disadvantages and limitations.

I have discovered that it is possible to case-harden steels and like metals in a sodium cyanide bath without the disadvantages of the prior art methods and compositions. By my invention I am able to produce a deeper case in less time than was heretofore possible with baths of this character. This is done by using a molten bath containing very small percentages of sodium cyanide and including a mixture of alkali metal and alkali earth metal halides, the latter in preponderance.

The following specific example is given as an illustration of my invention without in any way serving as a limitation thereof. The composition which is molten to serve as a case-hardening bath comprises a mixture of an alkali metal halide, an alkali earth metal halide, and a small amount of sodium cyanide, the alkali earth metal halide being present in preponderance. More specifically, I make a mixture containing one part by weight of sodium chloride and two parts by weight of calcium chloride. This mixture is dried and is ready for use in the melting pot or the like. After the mixture is molten, there is added sodium cyanide in the amount of  $\frac{1}{2}$  to 1% of the total bath. With a bath consisting of 100 lbs. of the mixed chlorides, I add  $\frac{1}{2}$  to 1 lb. of sodium cyanide. The bath is operated in the usual manner and, in accordance with the usual practice, the sodium cyanide is replaced as it is consumed. In ordinary operation, I add about  $\frac{1}{2}$  to 1% sodium cyanide per hour. Likewise, the efficacy of the bath can be maintained by the addition of suitable quantities of the chlorides, as necessary.

With the bath just described, maintained at a temperature of  $1525^{\circ}$  F., a case of 0.007 inch was produced on low carbon steel in fifteen minutes.

With a bath containing 40% sodium cyanide and the balance consisting of sodium carbonate and sodium chloride also maintained at  $1525^{\circ}$  F., similar low carbon steel was given a case of 0.005 inch in twenty-five minutes. Similar superior results are obtained at different times and temperatures using various grades of steel.

The sodium cyanide used may be the ordinary commercial grade containing 96% to 98% pure sodium cyanide, although other grades may be used in place thereof. I may prepare a special mixture by the fusion of sodium cyanide with calcium chloride and sodium chloride in such proportions as to maintain the desired ratio of the three constituents of the bath. The fused materials may be cooled and cast in the form of blocks convenient to handle, or may be prepared in any other suitable form.

While many theories and explanations may suggest themselves to those skilled in the art to account for the improved results obtained by me, it would appear that the superiority of my bath may be explained as follows. Sodium cyanide decomposes in the usual case-hardening bath and forms sodium carbonate and carbon monoxide, the latter serving to carburize the surface of the steel. However, sodium carbonate decarburizes steel and a point is reached where the tendency for the sodium carbonate to remove carbon from the steel exceeds the rate at which sodium cyanide adds carbon thereto. This equilibrium can only be overcome by the use of high concentrations of sodium cyanide in the bath with the obvious disadvantages of such an inefficient procedure.

In my bath, such sodium carbonate as may be formed can be removed from the bath or is prevented from decarburizing the steel by the use of the alkali earth metal halide such as calcium chloride. These latter compounds form insoluble alkali earth metal carbonates or oxides according to the temperature of operation, and the carbonate or oxide is either dissolved in the excess alkali earth metal halide or if some of it fails to dissolve, it will be found to sink to the bottom of the molten bath as a sludge and can be removed by means of a ladle or the like. Of course, it is understood that I do not wish to restrict myself to this theory of operation, although it would appear to account for the marked efficiency and superiority of my bath.

It will be apparent that many changes and variations other than those described can be made in the composition of the bath, as well as in the

case-hardening procedure without departing from the spirit and scope of the invention.

I claim:

1. A molten bath for case-hardening metals comprising essentially not substantially over 1% of sodium cyanide and a mixture of salts including an alkali earth metal chloride and an alkali metal chloride, the alkali earth metal chloride forming at least 50% of the mixture.

10 2. A molten bath for case-hardening metals comprising essentially not substantially over 1% of sodium cyanide and a mixture of salts including an alkali earth metal chloride and an alkali metal chloride in the proportion of two parts alkali earth metal halide to one part alkali metal chloride.

15 3. A molten bath for case-hardening metals comprising essentially  $\frac{1}{2}$  to 1% sodium cyanide and a mixture of salts including an alkali earth metal chloride and an alkali metal chloride, the alkali earth metal chloride forming at least 50% of the mixture.

20 4. A molten bath for case-hardening metals comprising essentially  $\frac{1}{2}$  to 1% sodium cyanide and a mixture of salts including an alkali earth metal chloride and an alkali metal chloride in the proportion of two parts alkali earth metal chloride to one part alkali metal halide.

30

80

35

85

40

90

45

95

50

100

55

105

60

110

65

115

70

120

75

125

5. A molten bath for case-hardening metals comprising essentially not substantially over 1% sodium cyanide with a mixture of salts including calcium chloride and an alkali metal chloride, the calcium chloride forming at least 50% of the mixture.

6. A molten bath for case-hardening metals comprising essentially not substantially over 1% sodium cyanide with a mixture of salts including calcium chloride and an alkali metal chloride, in the proportion of two parts calcium chloride to one part alkali metal chloride.

7. A molten bath for case hardening metals comprising essentially  $\frac{1}{2}$  to 1% of sodium cyanide with a mixture of salts including calcium chloride and sodium chloride in the proportion of about two parts calcium chloride to one part sodium chloride.

8. A molten bath for case-hardening metals comprising essentially a mixture of salts including an alkali earth metal chloride and sodium chloride in the proportion of approximately 2 parts of alkali earth metal chloride to 1 part of sodium chloride, and a minor portion of sodium cyanide as a case-hardening agent.

90

95

100

ERNEST C. MOFFETT.

105

110

115

120

125

130

135

140

145

150